

Patented May 19, 1925.

1,538,351

# UNITED STATES PATENT OFFICE.

CLARENCE RUDOLPH REIERSON, OF HAVRE, MONTANA.

## COLORING PHOTOGRAPHS.

No Drawing. Application filed August 2, 1922, Serial No. 579,244. Renewed April 1, 1925.

To all whom it may concern:

Be it known that I, CLARENCE RUDOLPH REIERSON, a citizen of the United States, residing at Havre, in the county of Hill and

5 State of Montana, have invented new and useful Improvements in Coloring Photographs, of which the following is a specification.

This invention relates to the decoration 10 of photographs and particularly to the production of oil colored photographs. Among other features the invention is directed to the use of particular materials and to the steps in the process by which the materials 15 are prepared, and to the particular sequence in which the materials are used in coloring photographs with oil colors.

One purpose of the invention is to reduce 20 the time necessary to complete the application of oil colors to a photographic print. Another purpose is to make possible a more even blending of oil colors than has heretofore been known. Another purpose is to provide a lustrous finish for photographic 25 prints without destroying the soft tone of the print. Finally the invention enables the artist to work rapidly without the smearing of oil colors, and makes it possible to complete the work in a remarkably short time.

30 Heretofore to complete the coloring of an average sized photographic print it has not been possible in less than from one to three hours, and after the completion of the coloring step two or three days have been usually required to properly dry the work. The details of the present invention enable the average artist to color with oil paint a photograph in fifteen or twenty minutes, and the work thus completed will dry within 35 seven to ten hours. Thus a dozen photographs could be colored in oil in one evening, and could be dry by morning, when they are in condition for mounting and delivery to the purchaser.

40 The invention includes three chief essential features which are as follows.

First, the materials and the process of preparing the materials into a composition for application directly to the photographic 45 print.

Second, the process of preparing the photographic print with the completed material of the first feature in order to make the print ready for receiving the decorative paint coating.

50 Third, the materials and the process of

preparing the mixture of the same for the outer and final protective coating which is applied to the decorative paint coats.

The details of these three features will 60 now be described.

The first feature, which includes the preparation and materials for the initial treating material, relates to a liquid, which, when properly applied, produces an oil 65 body surface upon photographic prints, which surface is suitable for the reception and blending thereon of artists' oil colors such as are usually sold in tubes.

To make the liquid of feature one, the 70 following ingredients, in the following proportions, are mixed in accordance with the steps specified. 3 parts of raw linseed oil, 3 parts of Japanese drier, and 2 parts of commercial ether are used. The Japanese drier is added to the oil and thoroughly mixed. To the resultant product the specified proportion of ether is added, and the resultant material is thoroughly mixed. Care should be taken to use substantially the 75 proportions and sequence specified because a perfectly acting solution may be prepared in this way, but if the proportions and order of treatment are materially disregarded, undesirable precipitates may be formed and 80 the materials spoiled.

The treatment of the photographic print should be conducted substantially according to the following details. The solution, prepared in accordance with feature one, should 85 be applied to the surface of the print with a tuft of cotton or some other equally soft material, and any surplus solution, which has not been absorbed by the emulsion on the print must be removed by rubbing the 90 damp surface with a piece of dry soft cotton fabric. The solution acts upon the photographic print in substantially the following manner. The ether of the solution permits the introduction into the emulsion of the 95 print of the required quantity of oil and Japanese drier. Probably the action is one in which the ether opens the pores of the emulsion, or otherwise so prepares it, so as to permit the introduction of the oil and drier, or at least permits a unified combination of the oil and drier with the material of the emulsion. The ultimate effect, regardless of the theory of the action, is that the material sizes the emulsion, or so prepares it, as to make possible the application 100 and blending thereon of artists' oil colors 105 110

in tubes evenly, smoothly, and without smearing, all to a degree of perfection heretofore not possible before the use of the particular solution mentioned. When oil colors are applied to a print or to an emulsion to which oil has been applied in a manner different from that above described, the application of the material is not even or smooth, the oil rubs off and smears, and the oil colors also tend to rub off and smear.

The Japanese drier, probably augmented by the action of the ether, serves to make possible unusual rapidity on the part of the artist who is applying the oil colors because the artist is enabled to have the oil colors under control at all times, and also because the completed work dries rapidly. The drying qualities are just such as to cause the colors to take hold without running or smearing, and yet the colors do not set so rapidly as to take the control of the work out of the artists' hands.

Feature three, relating to the protective coating, will now be described. This material is intended for use as a protective lustre producing material for application directly over the oil colored photograph. The object of this feature of the invention is to provide a liquid, which when properly applied to a completed oil colored photograph, adds the desired lustre and gives to it an unnoticeable, even, protective covering. To make this solution 5 parts of raw linseed oil and 1 part of Japanese drier are thoroughly mixed. The material is applied to the decorative paint coat on the photographic print by the use of a tuft of cotton, and any surplus solution must be removed by rubbing gently with a similar dry tuft of cotton. The effect of the application of the protective coating is the production of a rapidly drying, unnoticeable coating which protects against dust, dirt, and the fading of the color coat. The desired lustre may thus be added to the completed work of the color coat without destroying the softer tones of the colored photograph. The same advantageous results obtained by using the protective coat may be accomplished by using the solution upon black and white, or sepia prints, as have been described by using the material over prints finished in oil colors.

The various features of this invention may be used, and the materials of each of the solutions may be applied effectively, in the treatment of matt, semi-matt, or gloss photographic prints, as well as in the making of Doretypes.

By following the details of the present invention a photographic print may be colored and the coloring protected so that the final product has such a perfect blending of color that the lines of the colors and the material of the protective coat are im-

perceptible. In addition to the proper blending, the time for the coloring is reduced to one-fifth to one-eighth of the time ordinarily required prior to the use of the initial treatment solution.

70

I claim:

1. The process of treating photographs to prepare them for coloring which process comprises treating the emulsion of a developed positive print with a coating of a material which includes raw linseed oil, Japanese drier, and ether.

75

2. The process of preparing colored photographs which process comprises treating the emulsion of a developed positive print with a primary coating of a material which includes raw linseed oil, Japanese drier, and ether, removing excess material of said primary coating, and applying over said primary coating a decorative oil paint coat.

80

3. The process of preparing colored photographs which process comprises treating the emulsion of a developed positive print with a primary coating of a material which includes an oil, a liquid drier, and ether, applying over said primary coating a decorative oil paint coat, and coating said decorative coat with an outer liquid material which includes an oil and Japanese 95 drier.

90

4. The process of preparing colored photographs which process comprises treating the emulsion of a developed positive print with a primary coating of a material which includes raw linseed oil, Japanese drier, and ether, removing excess material of said primary coating, applying over said primary coating a decorative oil paint coat, and coating said decorative coat with an outer liquid material which includes an oil and Japanese drier.

100

5. The process of preparing colored photographs which process comprises treating the emulsion of a developed positive print with a primary coating of a material which includes raw linseed oil, Japanese drier, and ether, applying over said primary coating a decorative oil paint coat, and coating said decorative coat with an outer liquid material which includes an oil and Japanese 115 drier.

110

6. The process of preparing colored photographs which process comprises treating the emulsion of a developed positive print with a primary coating of a material which includes an oil, a liquid drier, and ether, applying over said primary coating a decorative oil paint coat, and coating said decorative coat with an outer liquid material 120 which includes 5 parts of raw linseed oil and 1 part of Japanese drier.

125

7. The process of preparing colored photographs which process comprises treating the emulsion of a developed positive 130

print with a primary coating of a material which includes an oil, a liquid drier, and ether, removing excess material of said primary coating, applying over said primary coating a decorative oil paint coat, and coating said decorative coat with an outer liquid material which includes 5 parts of raw linseed oil and 1 part of Japanese drier.

8. The process of preparing colored photographs which process comprises treating the emulsion of a developed positive print with a primary coating of a material which includes raw linseed oil, Japanese drier, and ether, removing excess material of said primary coating, and immediately

applying over said primary coating a decorative oil paint coat.

9. The process of treating photographic prints which process comprises applying to a photograph a mixture of an oil, a liquid drier, and ether.

10. The process of preparing colored photographs, which process comprises treating the emulsion of a developed positive print with a mixture of an oil, a liquid drier, and ether, and applying to the print so treated a decorative coloring medium.

In testimony whereof I affix my signature.

CLARENCE RUDOLPH REIERSON.